

## UNITED STATES PATENT OFFICE

2,560,876

## METHOD FOR PURIFYING ROSIN

William G. Knox and George L. Deniston, Dayton, Ohio, assignors, by mesne assignments, to Howard M. Hempstead and Louise M. Hempstead, both of Mobile, Ala.

No Drawing. Application July 5, 1949,  
Serial No. 103,174

14 Claims. (Cl. 260—111)

1

This invention relates to a method of treating rosin. More particularly it relates to the purification of rosin by extractive methods.

Still more particularly it relates to a method for removing dark colored material from wood rosin to lighten its color.

Rosins of the trade are judged for purity by the lightness of their color. Those having clear bleached straw color are called WW or water white rosins and command a premium price.

Near the bottom of the rating scale are the FF and G rosins which are dark and black-brown in color. These dark colored rosins constitute a large percentage of the rosin yield from present manufacturing procedures.

In order to obtain higher yields of premium grade rosins, the crude rosins have been subjected to such treatments as precipitation of a portion of the rosin by the use of strong acids and alkalis, absorption of color bodies by diatomaceous earth, activated charcoal and the like, vacuum distillation, liquid phase extraction, or by a combination of various of the above methods.

All of the above mentioned methods have objectionable features, most important of which are loss of product, cost of reagents, non-recoverability of the reagents, time consuming nature of filtration steps when removing absorbents and precipitates from viscous, sticky rosin mixtures.

One process has been patented which involves extraction of rosins with liquid agents, but has met with indifferent success, and as far as we know has received only limited acceptance in the industry, because of the cost of reagents, such as furfural and methyl carbitol and the heavy losses of these reagents.

In these processes after the color body solvent has extracted a portion of the color bodies from the naphtha solution of rosin, the solvent solution is removed to recovering units where the solvent is separated and recovered by distillation.

Due to inability to remove all of the solvent from the residue, large losses of solvent with consequent heavy operating costs are incurred. The losses when attempting to utilize methyl carbitol, which boils at about 380° F., have been such as to class this process out of the competitive market.

It is the primary object of this invention, therefore, to provide a process for the purification of wood rosin which overcomes the disadvantages of processes utilized heretofore.

2

It is an object of this invention to use a solvent for rosin which is inexpensive and whereby any losses incurred will not greatly add to the cost of processing.

It is another object of this invention to provide a process capable of producing a greater color improvement in wood rosins than has been evidenced heretofore.

Another object of this invention is to provide a process wherein the steps are adaptable to batch or continuous operation.

A still further object of this invention is to provide a process wherein the more expensive reagents are merely transfer agents and as such recoverable for recycling through the various process steps without appreciable loss.

It is another object of this invention to provide a process in which the operating costs are reduced because of the smaller volume of liquids which may be recycled in the various process steps.

In accordance with a process disclosed in the co-pending application of Cunningham and Knox, Serial No. 94,852, filed May 23, 1949, there is formed and separated several combinations of miscible solvents which are separable into homogeneous solution phases from which product and solvent are relatively completely separated and recovered.

By this process a major portion of the rosin product is recovered as upgraded higher value rosin and a minor portion of the rosin is recovered as dark low grade rosin.

Advantage is taken in this process of the discovery that, for example, diethylene glycol monomethyl ether has limited solubility in naphtha, whereas naphtha is slightly soluble in the ether, and in combination therewith makes an effective medium for accumulation of soluble color bodies.

The process is simplified by the discovery that the naphtha and color bodies are rendered insoluble in the ether solution diluted with water.

In brief, the process is carried out by preparing a solution of rosin in a primary solvent and extracting the primary solvent solution with a secondary solvent in which the primary solvent has limited solubility, to form a two phase system in which the mixed solvent phase preferentially dissolves the color bodies, effecting phase separation between primary and secondary solvent solutions by diluting the mixed solvent phase with an agent miscible with the secondary solvent and relatively completely recovering the various components of the segregated solution by distillation.

Several combinations of solvents and springing agents may be used. In the preferred embodiment, explained in more detail, the combination comprises naphtha as a primary solvent, ethylene glycol monomethyl ether as a secondary solvent, and water as a springing agent.

Other materials useful as primary solvents are hydrocarbons and hydrocarbon distillates, such as benzene, toluol, solvent acetates, and the like.

We have found it possible to use as secondary solvents alcohol-ethers, such as diethylene glycol monoethyl ether, alcohols such as tetrahydrofurfuryl alcohol, amino-alcohols such as 2-amino-1-propanol, 2-amino-1-butanol.

Springing agents utility depends upon the completeness with which the agent removes secondary solvent from the phase in which it is found. When utilizing alcohol ethers, alcohols and the like as secondary solvents, water serves as an inexpensive and efficient agent.

Inasmuch as the springing agent is merely recycled complete separation from the solvent is unnecessary. It is preferred, however, to choose springing agents which are separable into a recycle stream containing less than 5 percent of solvent.

Our modification of this process is based upon the discovery that by carrying out the extraction part of the process under the hereinafter described conditions, the performance of this system may be altered to such an extent that not only can the quantity of solvent which must be recirculated be markedly reduced, but a more complete removal of color bodies can be effected, so that a higher rating for rosin can be produced.

The economy of an extraction system naturally depends upon the relative quantities of solvents which must be circulated. In our improved system the first extraction step is carried out as follows:

The solution of rosin in primary solvent is mixed with secondary solvent. The mixture is warmed to a point where a homogeneous mixture is formed. The solution generally is heated to a temperature in the range of 85° F. to 150° F., and preferably to a temperature in the range of 90° F. to 110° F.

After agitation for about 15 minutes the solution is cooled to a temperature in the range of 0° to 65° F., although temperatures slightly outside this range may be utilized without lowering the efficiency of the system to too great an extent. For economic reasons it is preferred to operate the extraction step at about 45° F. to 60° F., and particularly at about 50° F.

The concentration of rosin in the primary solvent solution fed to the extraction stream is limited to between 5 and 30 percent by weight of rosin, preferably in the range of 10 to 20 percent.

The concentration of color bodies is generally limited to a maximum of about 20 percent by weight in the mixed solvent phase. Concentrations below 10 percent are considered poor operation in treating a crude rosin.

If, however, the process is carried out by repeated extractions, naturally the concentration of color bodies after the first extraction would not reach 10 percent with any appreciable circulation of secondary solvent, and therefore the invention is not tied to a lower limit.

For each volume of primary solvent and rosin fed to the extracting system, in our modified

process, we circulate about one-twelfth to one-sixth of a volume of secondary solvent. This solvent ratio, however, may be varied somewhat depending upon the contamination of the rosin.

In the solvent springing step we have found the separation of phases and transfer of color bodies to be more complete and efficiently performed when the step is carried out in a temperature in the range of 45° F. to 65° F. and preferably at a temperature of about 50° F., although temperatures outside the above range do not alter the separation efficiency as markedly as rise in temperature affects the efficiency of the extraction step.

In this cold water washing step the volume of water required is such that about one-fourth to one-half volume of springing agent is required for each volume of ether solvent solution.

The method of operation will be more clearly understood from the description in the following examples:

#### Example I

A batch of FF rosin, for example, weighing 1000 grams may be dissolved in about 5000 cc. of a mixture of pentane and hexane. This solution may be thoroughly mixed with 600 cc. of diethylene glycol mono ethyl ether, fed to the mixing chamber at a temperature of about 150° F. The temperature after mixing will be about 100° F. for the whole batch. The mixture may then be cooled by passing brine through cooling coils in the mixing vat until the temperature of the mixture is reduced to about 50° F.

The light colored rosin mixture may be segregated as a light colored solution and distilled at about 150° F. to recover the pentane solvent.

The dark colored solution may be mixed with approximately 400 cc. of water. After allowing the solutions to settle, this solution divides into a second pentane rosin solvent solution of about 300 cc. volume, containing substantially all of the color bodies.

The pentane solvent may be distilled from this solution at about 150° F. A volume of about 1000 cc. of alcohol-water solution is recovered and rectified at a temperature of about 212° F. to drive off the water which is condensed and reused in the water wash or springing step.

#### Example II

A solution of FF rosin, for example, having a ratio of one gram of rosin for each 5 cc. of solvent naphtha may be continuously processed as follows:

The solution may be continuously mixed with one volume of tetrahydrofurfuryl alcohol for each six volumes of naphtha solution.

The mixture may be heated to approximately 110° F. and run through suitable reaction timing equipment to allow a reaction time of approximately 15 minutes.

The homogeneous stream of solution issuing from the timing equipment may then be introduced into phase separation equipment wherein the solution is cooled to approximately 45° F.

From the top of this equipment there is continuously removed a clear rosin rich naphtha solution, and from the bottom of this equipment is continuously removed a dark alcohol rich solution.

The effluent top stream of light colored naphtha solution may be distilled at approximately 175° F. to recover the naphtha and light colored rosin separately.

The dark colored alcohol solution may then be run in a downward current flow to a wash tower. To the bottom of this wash tower may be fed one volume of water for each two volumes of alcohol solution entering at the top.

The naphtha-rosin color body solution withdrawn from the bottom of the wash tower may then be distilled at about 175° F. with the aid of a slight vacuum to recover the naphtha.

The alcohol-water solution issuing from the top of the tower may then be distilled at about 215° F. to remove water which is condensed and reused in the system. The collected naphtha and ether may then be recycled in the extraction system. The improvement in the process will be apparent from the following comparative data:

5. The method of removing color bodies from a solution of low grade rosin which comprises, mixing a solution of rosin in a water immiscible primary solvent with a secondary water miscible solvent having solvent power for the color bodies, 10 agitating and warming the mixture until a homogeneous solution is formed, cooling said solution to produce two separate solution phases, segregating said phases, springing secondary solvent from each phase by addition of water thereto, 15 segregating a pale rosin solution, a dark rosin solution, and a springing agent-secondary solvent

| Process             | Starting Material | Rosin Product Rating | Extraction Step Temperature | Temperature at Phase Separation | Volume Ratio in extraction step |
|---------------------|-------------------|----------------------|-----------------------------|---------------------------------|---------------------------------|
| Countercurrent..... | FF Rosin          | K                    | 73                          | 73                              | 1:0.25                          |
| Batch.....          | FF Rosin          | L                    | 100                         | 50                              | 1:0.15                          |
| Countercurrent..... | FF Rosin          | N                    | 100                         | 60                              | 1:0.10                          |

It will be understood that while there have been given herein certain specific examples of the practice of this invention, it is not intended thereby to have this invention limited to or circumscribed by the specific details of materials, proportions, or conditions herein specified, in view of the fact that this invention may be modified according to individual preference or conditions without necessarily departing from the spirit of this disclosure and the scope of the appended claims.

We claim:

1. The method of removing color bodies from solutions of low grade rosin which comprises, mixing a solution of rosin in a water immiscible primary solvent with a secondary water miscible solvent having solvent power for the color bodies to form a homogeneous solution, segregating a primary solvent rich phase and a secondary solvent rich phase, springing said secondary solvent from each phase by addition of water thereto, segregating a pale rosin solution, a dark rosin solution and a springing agent-secondary solvent solution, and recovering the solvents and springing agent for reuse in the system.

2. The method of removing color bodies from a solution of low grade rosin which comprises, mixing a solution of rosin in a water immiscible primary solvent with a secondary water miscible solvent having solvent power for color bodies to form a homogeneous solution, effecting phase separation by cooling said solution, separating secondary solvent from each phase by addition of water thereto, segregating two separate rosin solutions and a secondary solvent-springing agent solution, and recovering the individual liquids for reuse in the system.

3. The method of removing color bodies from a solution of low grade rosin which comprises, mixing a solution of rosin in a water immiscible primary solvent with a secondary water miscible solvent having solvent power for the color bodies to form a homogeneous solution, cooling the mixture to effect separation of a pale rosin phase and a secondary solvent rich phase, springing the contaminated quantity of secondary solvent from the pale phase by addition of water to said phase, segregating a pale rosin-primary solvent solution from the springing agent-secondary solvent solution, mixing water with the secondary solvent rich

phase to produce immiscible phases therein, segregating the immiscible phases, and heating each segregated solution to recover the individual liquids for reuse in the process.

4. The method of removing color bodies from a solution of low grade rosin which comprises, mixing a solution of rosin in a water immiscible primary solvent with a secondary water miscible solvent having solvent power for the color bodies, 10 agitating and warming the mixture until a homogeneous solution is formed, cooling said solution to produce two separate solution phases, segregating said phases, springing secondary solvent from each phase by addition of water thereto, 15 segregating a pale rosin solution, a dark rosin solution, and a springing agent-secondary solvent

solution, and separately recovering the solvents and springing agent for reuse in the system.

5. The method of removing color bodies from a solution of low grade rosin which comprises, mixing a solution of rosin in a water immiscible primary solvent with a secondary water miscible solvent having solvent power for the color bodies, 30 agitating and warming the mixture to a temperature in the range of 85° F. to 150° F. whereby a homogeneous solution is formed, cooling said solution to produce two separate solution phases, segregating said phases, springing secondary solvent from each phase by addition of water thereto, 35 segregating a pale rosin solution, a dark rosin solution, and a springing agent-secondary solvent solution, and separately recovering the solvents and springing agent for reuse in the system.

6. The method of removing color bodies from a solution of low grade rosin which comprises, mixing a warm solution of rosin in a water immiscible primary solvent with a warm secondary water miscible solvent having solvent power for the color bodies, agitating the mixture until a 40 homogeneous solution is formed, cooling said solution to produce two separate solution phases, segregating said phases, springing secondary solvent for each phase by addition of water thereto, 45 segregating a pale rosin solution, a dark rosin solution, and a springing agent-secondary solvent solution, and separately recovering the solvents and springing agent for reuse in the system.

7. The method of removing color bodies from a solution of low grade rosin which comprises, mixing a solution of rosin in a water immiscible primary solvent with a secondary water miscible solvent having solvent power for the color bodies, 50 agitating and warming the mixture to a temperature in the range of 90° F. to 110° F. whereby a homogeneous solution is formed, cooling said solution to produce two separate solution phases, 55 segregating said phases, springing secondary solvent for each phase by addition of water thereto, segregating a pale rosin solution, a dark rosin solution, and a springing agent-secondary solvent solution, and separately recovering the solvents and springing agent for reuse in the system.

8. The method of removing color bodies from a solution of low grade rosin which comprises, mixing a solution of rosin in a water immiscible

primary solvent with a secondary water miscible solvent having solvent power for the color bodies to form a homogeneous solution, cooling said homogeneous solution to a temperature in the range of 0° F. to 65° F., segregating a primary solvent rich phase and a secondary solvent rich phase, springing said secondary solvent from each phase by addition of water, segregating a pale rosin solution, a dark rosin solution and a springing agent-secondary solvent solution, and recovering the solvents and springing agent for reuse in the system.

9. The method of removing color bodies from solutions of low grade rosin which comprises, mixing a solution of rosin in a water immiscible primary solvent with a secondary water miscible solvent having solvent power for the color bodies to form a homogeneous solution, cooling said homogeneous solution to a temperature in the range of 45° F. to 60° F., segregating a primary solvent rich phase and a secondary solvent rich phase, springing said secondary solvent from each phase by addition of water thereto, segregating a pale rosin solution, a dark rosin solution, and a springing agent-secondary solvent solution, and recovering the solvents and springing agent for reuse in the system.

10. The method of removing color bodies from a solution of low grade rosin which comprises, mixing a solution of rosin in a water immiscible primary solvent with a secondary water miscible solvent having solvent power for the color bodies, agitating and warming the mixture to a temperature in the range of 85° F. to 150° F. until a homogeneous solution is formed, cooling said solution to a temperature in the range of 0° to 65° F. to produce two separate solution phases, segregating said phases, springing secondary solvent from each phase by addition of water thereto, segregating a pale rosin solution, a dark rosin solution, and a springing agent-secondary solvent solution, and separately recovering the solvents and springing agent for reuse in the system.

11. The method of removing color bodies from a solution of low grade rosin, which comprises dissolving the rosin in a mixture of pentane and hexane, mixing the solution with diethylene glycol monoethyl ether, agitating and warming the mixture to a temperature in the range of 85° F. to 150° F. until a homogeneous solution is formed, cooling said solution to a temperature in the range of 0° to 65° F. to effect separation of two distinct solution phases, segregating the light colored phase from the dark colored phase, mixing water with the light colored phase, segregating a diethylene glycol monoethyl ether-free pale rosin solution, mixing water with the dark phase, segregating a dark rosin solution and a water-diethylene glycol monoethyl ether solution, distilling the pentane-hexane solvent from the rosin solutions to recover a light and a dark rosin, and rectifying the diethylene glycol monoethyl ether solution to recover separately the ether and water components for recycling in the system.

12. The method of removing color bodies from a solution of low grade rosin, which comprises dissolving the rosin in a solvent naphtha, mixing the solution with tetrahydrofurfuryl alcohol, agitating and warming the mixture to a temperature in the range of 85° F. to 150° F. until a homogeneous solution is formed, cooling said solution to a temperature in the range of 0° to 65° F. to

effect separation of two distinct solution phases, segregating the light colored phase from the dark colored phase, mixing water with the light colored phase, segregating a tetrahydrofurfuryl alcohol-free pale rosin solution, mixing water with the dark phase, segregating a dark rosin solution and a water-tetrahydrofurfuryl alcohol solution, distilling the naphtha solution from the rosin solutions to recover a light and a dark rosin and naphtha, and rectifying the tetrahydrofurfuryl alcohol solution to recover separately the alcohol and water components for recycling in the system.

13. The method of removing color bodies from a solution of low grade rosin which comprises, dissolving one unit weight of rosin in five unit volumes of a mixture of pentane and hexane, mixing the solution with one volume of diethylene glycol monoethyl ether for each six volumes of solution, agitating and warming the mixture to a temperature of about 100° F., cooling the solution to a temperature of about 50° F. to effect separation of two distinct solution phases, segregating the light colored phase from the dark colored phase, mixing water with the light colored phase, segregating a diethylene glycol monoethyl ether-free pale rosin solution, mixing one volume of water with each volume of dark phase solution, segregating a dark rosin solution and a water-diethylene glycol monoethyl ether solution, distilling the pentane-hexane solvent from each of the rosin solutions to recover a light and a dark rosin, and rectifying the diethylene glycol monoethyl ether solution to recover separately the ether and water components for recycling in the system.

14. The method of removing color bodies from a solution of low grade rosin which comprises, dissolving one unit weight of rosin in five unit volumes of solvent naphtha, mixing the solution with one volume of tetrahydrofurfuryl alcohol for each six volumes of solution, agitating and warming the mixture to a temperature of approximately 110° F., cooling the solution to a temperature of approximately 45° F. to effect separation of two distinct solution phases, segregating the light colored phase from the dark colored phase, mixing water with the light colored phase, segregating a tetrahydrofurfuryl alcohol-free pale rosin solution, mixing one volume of water with two volumes of alcohol solution, segregating a dark rosin solution and a water-tetrahydrofurfuryl solution, distilling the naphtha solution from each of the rosin solutions to recover a light and a dark rosin, and rectifying the tetrahydrofurfuryl alcohol solution to recover separately the alcohol and water components for recycling in the system.

WILLIAM G. KNOX.

GEORGE L. DENISTON.

#### REFERENCES CITED

The following references are of record in the file of this patent:

#### UNITED STATES PATENTS

| Number    | Name   | Date          |
|-----------|--------|---------------|
| 2,117,572 | Rankin | May 17, 1930  |
| 2,325,410 | Lister | July 27, 1943 |
| 2,336,546 | Jones  | Dec. 14, 1943 |
| 2,336,547 | Jones  | Dec. 14, 1943 |